

Oct. 3, 1967

HIROSHI SHIBATA ET AL

3,345,283

PROCESS FOR PRODUCING A GRAPHITE ANODE

Filed June 5, 1963

2 Sheets-Sheet 1



FIG. 1.

FIG. 2.



FIG. 3.



FIG. 4.



FIG. 5.

INVENTORS

HIROSHI SHIBATA  
YASUO YAMASAKI  
KINZO SUGIHARA

BY *Bailey, Stephens & Huettig*  
ATTORNEYS

Oct. 3, 1967

HIROSHI SHIBATA ET AL

3,345,283

PROCESS FOR PRODUCING A GRAPHITE ANODE

Filed June 5, 1963

2 Sheets-Sheet 2



INVENTORS  
HIROSHI SHIBATA  
YASUO YAMASAKI  
KUNAO SUGIHARA

BY *Bailey, Stephens & Muetzel*  
ATTORNEYS

**1**

3,345,283

**PROCESS FOR PRODUCING A  
GRAPHITE ANODE**

Hiroshi Shibata, Yasuo Yamasaki, and Kinzo Sugihara, Nakoso, Fukushima Prefecture, Japan, assignors to Kureha Chemical Industry Co., Ltd., Tokyo, Japan, a corporation of Japan

Filed June 5, 1963, Ser. No. 285,771

Claims priority, application Japan, July 5, 1962,  
37/28,209, 37/37,061  
3 Claims. (Cl. 204—294)

**ABSTRACT OF THE DISCLOSURE**

A graphite anode for the electrolysis of alkaline salt solutions in an electrolytic cell having a mercury electrode is produced by impregnating the graphite electrode and coating the conductive connector pole composed of a metal having a lower electrical resistance than graphite, with a chlorine resistant material.

The present invention relates to a process for producing a graphite anode for an electrolytic cell used in the electrolysis of alkaline salt solutions by the mercury process.

An object of this invention is to produce a process for making an anode operable at a high current density.

Another object of this invention is to obtain anodes of low electrolyzing voltage at a high current density.

A further object of this invention is to produce durable anodes, wherein the amount of graphite consumption is less at a high current density.

Still another object of the present invention is to heighten the original unit of graphite.

A still further object of this invention is to increase the long-term continuous operation of an electrolytic cell by prolonging the interval for cleaning the electrolytic cell.

With regard to the graphite anode for an electrolytic cell for the electrolysis of alkyl salt solutions by the mercury process, the requirements for such graphite anode are that the graphite anode is resistant to nascent chlorine, has small overvoltage to chlorine, and is inexpensive, etc. However, the conventional graphic anode has the following defects. Namely, the graphite anode is not resistant to nascent oxygen and is porous, etc.

Hypochlorite ions, hydroxide ions and sulfate ions exist in an alkaline salt solution and these ions discharge, respectively, at the anode to evolve oxygen gas, and a part of these ions react directly with the graphite anode to generate carbon dioxide, and further destroys the bonding which binds together the fine particles constituting the graphite anode and finally the anode is mechanically crushed.

Thus, as the graphite anode consumes, fine and coarse pieces of the crushed anode fall onto the surface of the cathode amalgam and decompose the sodium amalgam to give rise to an evolution of hydrogen.

If a further large amount of graphite pieces fall onto the surface of the amalgam, the pieces will be mixed with sodium amalgam to form a mercury paste of high viscosity, and the paste will adhere to the surface of the cathode iron plate and stay thereat with the result that not only

**2**

the flow of mercury is hindered but also the amount of buried mercury in the electrolytic cell increases, and thus the flowing amount of mercury is lowered and the concentration of sodium amalgam is enhanced so that decomposition of the amalgam is promoted and the evolution of hydrogen will occur.

Accordingly, not only is the operation of the electrolytic cell seriously interrupted but also the current efficiency is markedly decreased, and if the concentration of sodium amalgam amounts to 1%, the cathode amalgam will lose entirely its fluidity and stick in a layer to the surface of the cathode iron plate to bring about an evolution of a large amount of hydrogen so that the electrolytic cell can explode.

Since the degree of consumption of graphite anode as described above increases with the increase of current density and rise of temperature in the electrolytic cell, and the amount of chlorine gas evolved from the lower surface of the anode increases proportionally to the current density, the mechanical destruction of the graphite anode by chlorine increases so that it shortens the life of the graphite anode and moreover the amount of fine particles of the crushed graphite anode is increased which fall onto the surface of the cathode amalgam.

On the other hand, since the anode graphite is porous, the electrolyte penetrates into the interior of the anode, and the supplying of chlorine ions is not sufficient in the pores of the anode so that discharge of hydrogen and sulfate ions is brought about, oxygen is evolved, and as a result, the anode is swollen and subjected to oxidation-consumption, and thus, the anode is deteriorated.

Such a detrimental and harmful effect is intensified with the rise of current density, the electric resistance of the graphite anode is increased, the electrolyzing voltage is increased, which results in a decrease of the original unit of electrolyzing power.

Reference is made to the anode pole to be connected to the graphite anode plate as follows:

There have hitherto been used many graphite poles, like a graphite anode plate, but this graphite is accompanied in this case by the following defects:

In the first place, in the case where the current density has become high, the graphite pole never stands the load with its inherent resistance, and heat generation and voltage losses become larger. Secondly, the contact resistance at the connected portion of the anode pole and the anode plate is so large that operation under a high current density becomes impossible. Thirdly, the graphite pole becomes aged and consumed in the electrolyte solution and must be discarded within a few months. Fourthly, the connected part of the anode pole with the anode plate is also corroded by the electrolyte solution and its electric resistance is increased in the course of its use. On account of the defects as described above, with regard to an anode pole adapted for operation under a high current density as much as about 100 amp./dm.<sup>2</sup>, it is necessary to establish a process for using a metallic pole having lower electric resistance than graphite, as well as for making an anode pole which can be completely connected to an anode plate where the said metallic pole is never corroded by salt water.

In order to accomplish the operation under an anode current density over 100 amp./dm.<sup>2</sup>, the present invention teaches that it is essentially important in the first place

that the anode has low electric resistance; in the second place, the anode is less consumed and has a protracted life and that in the third place the anode is not seriously aged over a long period of time.

In order to enable the invention to be more readily understood, reference is now made by way of example to the accompanying drawings which illustrate diagrammatically embodiments thereof, and in which:

FIG. 1 is a cross-sectional perspective view of an electrolytic cell for electrolyzing alkaline salt solutions by the mercury process, wherein graphite anodes produced according to this invention are set;

FIG. 2 is an enlarged view of a model, showing the internal structure of a conventional graphite anode;

FIG. 3 is an enlarged view of a model, showing the internal structure of a graphite anode according to this invention;

FIG. 4 is a perspective assembled view showing by way of example an embodiment of a graphite anode produced according to this invention;

FIG. 5 is a cross-sectional view taken on the line V—V in FIG. 4;

FIG. 6 is a perspective view showing by way of example another embodiment of a graphite anode produced according to this invention;

FIG. 7 is a cross-sectional view taken on the line VII—VII in FIG. 6;

FIG. 8 is a perspective view showing by way of example a further embodiment of a graphite anode produced according to this invention; and

FIG. 9 is a cross-sectional view taken on the line IX—IX in FIG. 8.

Referring to the drawing in detail, wherein like reference characters indicate like parts throughout the several figures:

In FIG. 1, the electrolytic cell is composed of a cell body having connecting side walls 1 provided with rubber lining joined to a cathode bottom plate 3 through the medium of rubber packing 2. The anode according to this invention is composed of anode plate 5 and anode connector pole 4, and is immersed in an electrolyte solution 7 with which the electrolytic cell is filled. Said anode is suspended and set through openings 12a of a cover plate 12 on the electrolytic cell at the distance of a few millimeters from the surface of the cathode amalgam layer 6. FIGURES 1 and 2 show that the anode plate 5 is composed of graphite particles 8. As shown in FIG. 1, the anode pole 4 is directly coated with a protective layer 13 composed of chlorine-proof material, such as hard rubber, synthetic resin or the like, and completely protected on its lower part from the electrolyte solution 7 by means of a protecting ring 14 composed of chlorine-proof material such as carbate, hard rubber, polyester resin, vinyl chloride resin and furan resin, carbon cement, powdered porcelain and graphite.

FIG. 2 is an enlarged view of a model showing the internal texture of a hitherto known graphic anode, and as can be seen therefrom, the pores of the graphite plate are completely embedded and filled with synthetic resin, and consequently, when such a graphite is used in electrolysis the graphite readily cracks due to the swelling of the resin.

FIG. 3 is an enlarged view of a model showing the texture of the anode plate according to the present invention, and the graphite particles 8 are bound or connected with each other by graphite tenacious bands 9. A film of synthetic resin latex is adhesively formed on the inner and outer walls of the boundary defined by the graphite particles 8 and tenacious bands 9, and spaces 10 are formed in the interior of the said boundary by evaporation of the said resin latex.

FIG. 4 is a perspective view showing one embodiment of the anode of the present invention, and in this figure the anode pole 4 having a protective layer 13 is connected to the anode plate produced by the specific treat-

ment as described hereinafter through a protective ring 14 made of chlorine-proof material. Furthermore with regard to this graphite anode pole, this anode connector pole can be substituted by a metallic anode pole made of metal, such as copper or brass, having lower electric resistance than that of the graphite. When such a metallic anode pole is employed, it is important to prevent the connected portion of the anode pole and the anode plate from the corrosion by the hot salt water containing chlorine.

FIG. 5 shows a sectional view taken on the line V—V of FIG. 4.

A tapered recess 16 is formed in the anode plate 5. The recess is then heated to about 150 to 200° C. A layer 17 subjected to the chlorine-proof treatment is formed by penetrating chlorine-proof chemicals such as chloronaphthalene, chloro-paraffin, chlorinated fish oil and vegetable oil into the anode plate under pressure or at reduced pressure from the inner part of the said recess. The anode connector pole 4, which has been covered with the protective layer 13 completely to the position corresponding to the top end of the tapered portion 15, is fitted into the said recess by pressing. Thereafter, the protective ring 14 is adhesively secured around the said protective layer 13 on the said anode plate 15 with a chlorine-proof adhesive agent as a base and the chlorine-proof adhesive agent 18 is further applied on the connected part between the anode pole and the anode plate so as to completely prevent the intrusion of salt water.

FIG. 6 is a perspective view showing another embodiment of the present invention. The anode pole 4 having the protective layer 13 is directly and firmly tightened to the anode plate by means of a screw-threaded ring 19 adjacent the protective ring 14.

FIG. 7 shows the structure of the sectional view taken on the line VII—VII of FIG. 6. The anode pole 4 is fitted into the anode plate 5 by means of the tapered end in the same way as in FIG. 5, but in this case, a screw-threaded ring 19 is disposed underneath the protective ring 14, and the lower bottom part of the protective layer 13 is provided with a threaded screw 21, on which the screw-threaded ring 19 is screwed. It should be noted that the connection between the anode pole and the anode plate is more fortified by the above-mentioned construction and the connected part is perfectly prevented from erosion by salt water. Namely, the anode pole 4 is integrally formed with the screw-threaded ring 19, and the said screw-threaded ring 19 is set on the anode plate 5 by a chlorine-proof adhesive agent 21. Since the protective ring 14 is further connected above the said screw-threaded ring 19 by means of chlorine-proof adhesive agent 18, the exfoliation of the anode pole 4 from the protective ring 14 by the thermal expansion due to the rise of temperature is completely prevented.

FIG. 8 is a perspective view, showing a further embodiment of the present invention. The anode pole 4 having the protective layer 13 is bolted to the anode plate 5 with aid of a ring 23 and bolts 22.

FIG. 9 shows the structure of the sectional view taken on the line IX—IX in FIG. 8.

As shown in FIG. 9, the anode pole 4 is fitted into the anode plate 5 with aid of a tapered end in the same way as in FIG. 5, however, the lower part of the protective layer 13 is directly provided with a threaded screw 13a and not only the ring 23 having bolts is screwed on this part but also bolt bores are formed in this ring 23, which is bolted on the anode plate 5 by means of bolts 22 made of chlorine-proof material. Between the ring 23 having bolts and the anode plate 5, the chlorine-proof adhesive 18 acts as a liquid packing. Accordingly, no exfoliation of the protective ring 23 from the anode plate 5 due to the thermal expansion of the anode pole 4 takes place and, moreover, since the anode pole 4 is secured to the anode plate 5 with aid of bolts 22, the supporting power by means of the anode pole 4 is much strengthened and the exfoliation of the

protecting ring 23 from the anode plate 5 due to the strain on the anode pole 4 is completely prevented and no intrusion of salt water takes place.

The anode plate produced by the specific treatment, which is the important point of this invention is further explained in detail as follows:

Some representatives of conventional processes for penetrating the pores of a graphite anode carried out heretofore for the purpose of covering the porosity which is the defect of graphite anode, diminishing the consumption of anode and enhancing the original unit of graphite so as to accomplish the long-term continuous operation of the electrolytic cell are described as follows:

Namely,

- (1) Filling the pores of a graphite anode with paraffin.
- (2) Filling the pores of a graphite anode with chlorinated oil.
- (3) Filling the pores of a graphite anode with chloro-naphthalene.

These known processes had great defects respectively and could only bring about some effect, and were successful in the anode of the electrolytic cell used in the diaphragm process, but could not be applied to the mercury process.

The mechanism of each of the said processes is described in detail below.

In the first place, in the case where the graphite anode is filled with paraffin, as shown in FIG. 2, the pores 10a defined or surrounded by graphite particles 8 and graphite bands 9 in the graphite anode are filled uniformly with paraffin. The consequence of the case where the anode is subjected to electrolysis in such a state, is explained below:

First, the temperature in electrolyte solution reaches as high as 80 to 90° C. in the case where the operation at high current density is popular these days. Accordingly, the paraffin in the inner part of the anode begins to melt and exudes in the bottom surface of the anode and simultaneously is converted into paraffin chloride by nascent chlorine, and thus, hydrochloric gas is generated with expansion of the volume so that the graphite is destroyed and concurrently therewith the said chloride itself falls on the surface of the cathode mercury and brings on the cause of an evolution of hydrogen.

In the second place, in case where the graphite anode is filled with chlorinated fish oil or chlorinated vegetable oil there takes place results similar to those in the case of paraffin, and the prevention of graphite integration due to the formation of protective film on the surface of the gradually chlorinated anode, which is the proper object, cannot be achieved.

Furthermore, in the case where the anode is filled with chloro-naphthalene, the exudation and chlorination of chloro-naphthalene is rather slow, but the following defects are caused:

That is, as shown in FIG. 2, since the pores are spaces 10a in the anode are completely embedded with chloro-naphthalene, the swelling thereof gives rise to cracks and crevices in the graphite texture, and the exfoliation occurs on the surface of the anode and large graphite particles fall.

And in this case, since the chloro-naphthalene has no effect to adhere to the surfaces of graphite particles and to include and bind the whole, the chloro-naphthalene promotes the further result in that the chloro-naphthalene exfoliates as a mixture with graphite pieces and falls from the anode onto the surface of mercury, and the evolution of hydrogen gas becomes violent.

Moreover, a carbate product is available on the market as graphite treated with synthetic resin but judging from the structure of the carbate product, extremely porous graphite is selected as a raw material and the pores thereof are perfectly filled with synthetic resin

to make the graphite into a concrete structure, and therefore it is the main object of the said carbate product to impart the resistance against chemicals to graphite as well as to prevent it from the leakage of chemicals. Accordingly, the heat conductivity and the anti-leakage properties of the product are excellent, but since the pores are completely filled with synthetic resin, in using this product in electrolysis the graphite cracks due to the swelling of synthetic resin embedded in the porous graphite and causes large particles which fall onto the surface of mercury to give rise to an evolution of hydrogen gas.

This invention completely overcomes all the defects of the conventional processes and creates the following process for preventing the anode from consumption:

Namely, the graphite anode having the structure as shown in FIG. 3 was obtained by using synthetic resin latex. Tenacious films 11 of synthetic resin having a thickness of 1 to 10 $\mu$  are formed adhesively on the inner and outer walls of anode pores while including and firmly binding the inner and outer surfaces of the graphite particles 8 and the tenacious bands 9, and thereby the swelling and disintegration of graphite is prevented.

Moreover, since the spaces 10 formed by evaporation of the water content in the resin latex do not cause cracks in the graphite by the swelling of the film of synthetic resin, and on account of electric non-conductivity of the film of synthetic resin a discharge of chlorine ions, hypochlorite ions and sulfate ions is prevented, and not only are the pores in the graphite free from disintegration but also the film can be formed by the least required amount of synthetic resin, and as the result the amount of synthetic resin to be used is considerably less as compared with that in conventional processes and the treatment of the anode becomes very economical and inexpensive.

Moreover, as regards the synthetic resin latex used in this invention, the said synthetic resin latex can be uniformly and completely applied to the inner and outer walls of pores in the anode graphite by a specific compounding, and this brings about a favorable result in that no formation of large graphite particles by exfoliation of the surface of the anode can take place over a long-term use of the anode, and the stabilization of the interpole adjustment of the anode and the rationalization of the feeding of electrical current to the anode as well as the enhancing of the electrolyzing voltage are achieved.

The synthetic resin latex used in this invention for the above-mentioned purpose has the following characteristics:

Namely, this resin latex is chlorine-proof and heat-resistant, has the property of forming a film at 80 to 90° C., does not decompose at 80 to 90° C. and has an excellent property for penetrating into the graphite anode pores.

Examples of the synthetic resin latex are exemplified as follows:

Copolymer or single polymer of vinylidene chloride, vinyl chloride, acrylonitrile and the like.

Furthermore, in order to improve the penetration of the resin latex, surface-active agents such as amionic soap, non-ionic soap and others may be added.

The resin concentration of the latex is preferably in the range of 5 to 50%, depending on the kind of graphite anode used and the conditions of use.

The process of causing synthetic resin to adhere to inner or outer walls of pores in graphite is described below:

Firstly, the anode is placed in a vacuum vessel and the air in the anode is evacuated, and then synthetic resin latex is poured into the vacuum vessel, and thereafter the interior of the vacuum vessel pressurized with the result that the tenacious resin latex film is caused to be adhesively formed on the inner and outer walls of pores, and binds the graphite particles and the tenacious bands.

With respect to the drying of the graphite anode after the latex coating, the temperature and the time of drying depend on the kind and the recipe of the synthetic resin, and the perfect adherence of the film of synthetic resin latex can be accomplished by drying at 50 to 100° C. for 4 to 10 hours.

Functions and effects of the anode treated by the process of this invention are described as follows:

In the first place, the film of synthetic resin latex formed in pores in the anode plate is excellent in chlorine-proof property and heat-resistance and can sufficiently be resistant to the shocks made by the rapid evolution of chlorine and oxygen from the surface of the anode when operating at high current density in the electrolytic cell, to disintegration due to swelling and shrinking of the anode caused by rapid change of temperature, and to mechanical abrasion due to the friction of chlorine gas on the surface of the anode.

In the second place, the anode of this invention is characterized in that the electric resistance of the whole anode is very low and the electrolyzing voltage when operating at high current density is extremely low.

Namely, metal having small electric resistance is used as an anode connector pole, a tapered end is used in the connection thereof to the electrolytic plate and moreover, as the result of laborious studies on tapering angle and fitting pressure, the contact resistance between the anode connector pole and the anode plate has been reduced to about one-fourth of that of a graphite pole so that no heat generation at the connected portion takes place even at a high current density about 100 amp./dm.<sup>2</sup>.

In the third place, in the structure of the connected portion between the anode connector pole and the anode plate, the tapered part is soaked with non-permeable and chlorine-proof material over its area and whole body from the inner surface of the tapered recess, and since the anode is constructed in such a way that it is not only prevented from the corrosion but also from strain and stress caused by thermal expansion, the anode of this invention has the feature of being capable of maintaining the electrolyzing voltage favorably over a long time.

In the fourth place, since the metallic anode pole is directly protected by the protective layer and consequently, the anode pole is preserved, and even in a case where the anode plate is consumed and discarded, the regeneration of the anode pole is possible if the protecting layer on the anode pole is renewed, and therefore about 0.5 kg./t. NaOH, calculated on the original unit of graphite, can be cut down, as compared with a graphite pole.

In the fifth place, the process for producing an anode according to this invention is characterized in that the process is rather simple as compared to its great effects, home-working is easy and the working cost is inexpensive.

The following is an example of this invention which gives a preferred form of forming the anode.

#### Example

Instance of the process for causing the synthetic resin latex to adhere firmly to the inner and outer walls of the pores in the graphite anode.

##### (1) Recipes of the resin latex used.

|                                                        | Percent |
|--------------------------------------------------------|---------|
| Vinylidene chloride monomer                            | 70      |
| Vinyl chloride monomer                                 | 30      |
| Concentration of resin                                 | 10      |
| Anionic soap (in a small but effective amount), added. |         |

##### (2) Process of working.

|                       |                      |              |
|-----------------------|----------------------|--------------|
| Vacuum degree         | mm. Hg.              | —600 to —700 |
| Time of sucking       | min.                 | 30-60        |
| Pressurized degree    | kg./cm. <sup>2</sup> | 3-4          |
| Temperature of drying | ° C.                 | 80           |
| Time of drying        | hrs.                 | 5            |

The results of using the anode worked by the process

according to the present invention are shown as follows, as compared with the conventional anode:

|                                                 | Articles | Conventional anode | Electrode of the present invention |
|-------------------------------------------------|----------|--------------------|------------------------------------|
| Passing current Kil. Amp.                       | 80       | 80                 |                                    |
| Current density Amp./dm. <sup>2</sup>           | 122      | 122                |                                    |
| Electrolyzing voltage (volt)                    | 5.0-5.1  | 4.5-4.6            |                                    |
| Temp. in electrolytic cell ° C.                 | 80-85    | 80-85              |                                    |
| Time of using the anode (days)                  | 8        | 16                 |                                    |
| Concentration of amalgam Na, percent            | 0.6      | 0.3                |                                    |
| Concentration of hydrogen in chlorine, percent  | 0.1-0.5  | 0-0.1              |                                    |
| Current efficiency, percent                     | 95       | 97                 |                                    |
| Interval of cleaning electrolytic cell (months) | 3-4      | 6-7                |                                    |
| Initial unit of graphite Kg./t. NaOH            | 3.5-4.0  | 2.0-2.5            |                                    |

What is claimed is:

1. In a process for producing a graphite anode in an electrolytic cell having a mercury electrode for the electrolysis of alkaline salt solutions the steps comprising in combination, respectively,
  - (a) forming a tapered recess in said graphite anode,
  - (b) heating the recess to about 150° C. to 200° C.
  - (c) under pressure depositing a chlorine resistant material in the recess, said material being selected from the group consisting of chloro-naphthalene, chloroparaffin, chlorinated fish oil, chlorinated vegetable oil and mixtures thereof,
  - (d) maintaining the said material and recess under pressure for about 30 to 60 minutes whereby the material penetrates into the graphite anode,
  - (e) forcing a conductive connector pole composed of a metal having a lower electrical resistance than graphite and having a tapered end into the recess with the tapered end fitting into the tapered recess in the graphite anode, any exposed part of the pole being coated with chlorine resistant material, and
  - (f) applying a chlorine resistant sealing protective ring composed of a material selected from the class consisting of impervious carbon, graphite, hard gum, polyester resin and vinyl chloride, and adhesive around the connector pole at the intersection of the pole and graphite anode
- 45 to form a graphite anode with a firmly bonded connector pole.
2. A process as in claim 1 wherein any exposed area of the connector pole is coated with at least one chlorine resistant compound selected from the group consisting of graphite, porcelain, carbon cement, furan resin, vinyl chloride resin, polyester resin and hard gum.
- 50 3. A process as in claim 1 wherein in step (f) at least one screw threaded protective ring consisting of chlorine resistant material is positioned under the said sealing protective ring to firmly hold the said pole in position.

#### References Cited

##### UNITED STATES PATENTS

|    |           |         |             |         |
|----|-----------|---------|-------------|---------|
| 60 | 508,091   | 11/1893 | Cutten      | 204—294 |
|    | 1,490,504 | 4/1924  | Bootman     | 204—286 |
|    | 2,069,862 | 2/1937  | Suzuki      | 204—290 |
|    | 2,328,665 | 9/1943  | Munson      | 204—250 |
|    | 2,649,411 | 8/1953  | Shat et al. | 240—266 |
| 65 | 2,820,728 | 1/1958  | Burns       | 204—294 |
|    | 2,920,004 | 1/1960  | Carlin      | 204—294 |
|    | 3,140,991 | 7/1964  | Gardiner    | 204—219 |
|    | 3,260,662 | 7/1966  | Henegar     | 204—279 |

##### OTHER REFERENCES

70 A.P.C. Application of Ott, Ser. No. 326,756. Published May 1943.

JOHN H. MACK, Primary Examiner.

75 D. R. JORDAN, Assistant Examiner.